

# UNITED STATES PATENT OFFICE.

THOMAS REGINALD DAVIDSON, OF WEMOUNT, QUEBEC, CANADA.

## METAL-PICKLING PROCESS.

1,104,107.

Specification of Letters Patent. Patented July 21, 1914.

No Drawing.

Application filed July 11, 1913. Serial No. 778,575.

To all whom it may concern:

Be it known that I, THOMAS REGINALD DAVIDSON, of the city of Westmount, Province of Quebec, Canada, have invented certain new and useful Improvements in Metal Pickling Processes; and I do hereby declare that the following is a full, clear, and exact description of the same.

This invention relates to the treatment of metal articles preparatory to receiving a coating of enamel or the like and has for its object to simplify and cheapen the process followed in such preparation and applies to articles made of sheet iron or steel or any other material which is not readily attacked by concentrated sulfuric acid at temperatures between 45° and 300° Fahrenheit.

In carrying out my process the metal articles just as they come, having on and in the surface thereof grease, fat, wax or other organic or foreign matter, from the die, are immersed for a period of about one minute in a bath of concentrated sulfuric acid heated to from 200°—300° Fahrenheit with the result that all the grease and other organic substances are carbonized and the articles when removed from the bath carry a film of the acid with the carbonized organic matter suspended therein. The most economical concentration is that of the common commercial sulfuric acid, of about 1.83 specific gravity and heated to about 200° Fahrenheit, but any concentration which will carbonize the grease, etc., is all that is required.

By heating the concentrated sulfuric acid to from 200°—300° Fahrenheit the process is more quickly performed but the same result may, if desired, be secured by immersing the articles a long time in relatively cold concentrated acid. The articles are then allowed to stand in water (preferably heated to about 150° Fahrenheit) and the concentrated acid becoming diluted loses its suspending quality and the carbonized matter is free to settle. The dilute acid remaining on the metal acts to further clean it of any adhering oxids as in the ordinary pickling process, and with its surfaces sufficiently cleansed the metal is removed from the water and further washed in clean water

heated preferably to near the boiling point after which the article is dried in the customary manner and is then ready to be enameled or otherwise coated.

What I claim is as follows:

1. The treatment of metal for cleansing the surface thereof preparatory to receiving a coating of enamel or the like, which consists in immersing same in concentrated sulfuric acid. 55

2. The treatment of metal for cleansing the surface thereof preparatory to receiving a coating of enamel or the like, which consists in first immersing same in concentrated sulfuric acid and then in a water bath. 60

3. The treatment of metal for cleansing the surface thereof preparatory to receiving a coating of enamel or the like, which consists in first immersing same in concentrated sulfuric acid, then in a water bath and subsequently washing the metal in a fresh bath of water. 65

4. The treatment of metal for cleansing the surface thereof preparatory to receiving a coating of enamel or the like, which consists in immersing such metal in heated concentrated sulfuric acid. 70

5. The treatment of metal for cleansing the surface thereof preparatory to receiving a coating of enamel or the like, which consists in first immersing such metal in heated concentrated sulfuric acid and then in a bath of heated water. 75

6. The treatment of metal for cleansing the surface thereof preparatory to receiving a coating of enamel or the like, which consists in first immersing such metal for about a minute in concentrated sulfuric acid heated to between 200° and 300° Fahr., then immersing the metal in a water bath heated to approximately 150° Fahr. and subsequently washing the metal in a fresh bath of water at about boiling point. 80

In testimony whereof, I have signed my name to this specification, in the presence of two subscribing witnesses. 85

THOMAS REGINALD DAVIDSON.

Witnesses:

STANLEY C. KING,

FRED J. SEARL.